

## UNITED STATES PATENT OFFICE

JEAN PAISSEAU, OF PARIS, FRANCE

## METHOD FOR VARNISHING LEATHER AND LIKE MATERIAL

No Drawing. Application filed October 19, 1925, Serial No. 63,569, and in France July 23, 1925.

The products in current use for the varnishing of leather and like material of animal or vegetable origin consist of complex coatings which are difficult of application and dry at a slow rate, such products always containing linseed oil which is variously treated with gums or resinous substances. Such varnishes are quite adhesive, but they can only be applied in thick layers, thus entirely concealing the underlying leather to which they give the uniform appearance of oil cloth.

It is further observed that a cellulose varnish of the known type, i. e. based upon the use of nitrocellulose or acetate of cellulose dissolved in the usual solvents, with or without the addition of a substance conferring plasticity, will not adhere to leather, and this is due to two reasons.

Firstly, the close grain of the cutaneous 20 derm constituting the leather will cause it to act as a semipermeable membrane, so that when the varnish is applied, the solvents alone will penetrate into the leather and the cellulose will not infiltrate between the fibres but 25 will remain on the surface in the shape of a film which fits closely upon all the reliefs but cannot adhere for lack of penetrating roots.

Secondly, the nitrocellulose or acetate of cellulose cannot adhere to the conjunctive 30 fibre of the leather from the fact that cellulose and its derivatives will not moisten the fibre. There is so to speak an incompatibility between these two substances, so that the nitrocellulose varnish will become detached 35 when the leather is bent or worked up or when it is immersed in water.

My invention has for its object to obviate such drawbacks, and it relates to improvements in the varnishing of leather in view of 40 imparting to them a glazed and brilliant surface equivalent to what is afforded by the known methods, but without change in the appearance or the quality of the leather. My said varnishing process is equally applicable 45 to wood, horn and like material.

For this purpose, the invention essentially consists in treating the leather so as to change 50 the nature of its surface whereby it will become united to the nitrocellulose of the varnish. I treat the leather for instance by a

superficial impregnation with gelatin or like organic substance which will adhere to the cellulose varnish or the like, which is then made insoluble by the tanning or other process.

The most simple process consists in the treatment of the surface of the leather to be varnished whereby it is partially converted into gelatin or analogous substance which is capable to adhere to the cellulose ethers.

To this end I may for example treat the leather with an organic or other acid diluted in a suitable solvent in order to graduate the action. I prefer to employ a volatile acid so as to avoid an excessively long action which would attack the leather at a too great depth and would thus reduce its strength in a prejudicial manner.

Among the acids which are preferable for this use, I may mention the following organic 70 acids: acetic, formic, lactic, tartaric, oxalic and like acids, or all other acids or bodies having an acid function, even if they are not miscible with the cellulose varnish, provided they will gelatinize the collagenic fibres of 75 the leather. The varnishing process is carried out in two stages; firstly, the preparation of the leather by the acid treatment, and secondly; when the leather is dry, the application of a suitable cellulose varnish.

Obviously the above cited acids may be replaced by any substances which are capable to give acid products by the chemical decomposition, either spontaneous or caused by the different elements which are in presence, that 85 is to say the constituent parts of the leather and of the varnish.

But I am enabled to operate in a more simple manner, and obtain the most approved results by adding the varnish to acetic acid 90 which has the advantage of being a solvent for nitrocellulose and acetate of cellulose, so that it may be incorporated into the varnish itself, thus simplifying the work, since the leather can be varnished in a single operation and no preliminary preparation is needed.

In practice, I find that the simplest and most rapid method consists in the use of a varnish based upon nitrocellulose for in- 100

stance, and comprising the usual solvents such as methyl amyl, or ethyl acetate, acetone, or the like; the proportion of nitrocellulose may vary according to circumstances between 2 and 6 per cent in order to afford the requisite fluidity.

To this varnish I add as a mordant a sufficient amount of concentrated acetic acid, according to the nature of the leather. In order to obtain the necessary suppleness and elasticity, I incorporate a substance conferring plasticity such castor oil or a derivative of the same which is not of a resinous nature, or any other suitable substance conferring plasticity which is of a stable and non-volatile nature.

According to the result to be obtained and the nature of the leather, I apply the varnish two or three times by means of a brush, a small scraper, an atomizer, or the like, and this will impart a brilliant glazed appearance to the leather without changing its aspect or its qualities.

As above stated, a varnish thus composed may be employed with approved results upon wood, horn or the like, and I further obtain an improvement which consists in forming upon the article a surface which is of a silky, velvety, lustrous or pearly nature and producing a most agreeable effect, by incorporating into a varnish a suitable quantity of pearl essence. The resulting effect will vary according to the amount of pearl essence employed, or according to the number of layers of varnish applied, and the material thus treated will constitute a new manufactured product which is susceptible of numerous applications.

Having thus described my process, what I claim as new therein, and my own invention, is:

1. A process for the varnishing of leathers and like substances, consisting in superficially gelatinizing the leather by the action of a suitable acid and in then covering this surface thus modified with a cellulosic varnish.

2. Process for the varnishing of the leathers and like substances which consists in gelatinizing the surface of the said leather by the action of a suitable acid and in coating this gelatinized leather with a layer of a varnish having cellulose ester as a base.

3. Process for the varnishing of the leathers and like substances which consists in gelatinizing the surface of the said leather in applying superficially a suitable acid diluted in a solvent and in then applying a varnish having cellulose ester as a base.

4. Process for the varnishing of the leathers and similar substances which consists in gelatinizing the surface of the said leather by applying superficially a suitable acid diluted in a solvent and in then applying a varnish based upon nitrocellulose to which

suitable substances conferring plasticity are added.

5. Process for the varnishing of the leathers and similar substances which consists in applying upon these substances a solution of a volatile acid capable of gelatinizing at least partially the collagenic fibre of the leather, then in applying upon the substances which have been treated in that way a cellulosic varnish to which a small quantity of acetic acid is added.

6. Process for the varnishing of the leathers and like substances which consists in applying upon these substances a solution of a volatile acid capable of gelatinizing at least partially the collagenic fibre of the leather, then in applying upon the substances which have thus been treated a cellulosic varnish containing acetic acid and plasticizing agent.

In testimony whereof I have hereunto affixed my signature.

JEAN PAISSEAU.

70

75

80

85

90

95

100

105

110

115

120

125

130